

# United States Patent [19]

Jayne et al.

[11] 3,994,948

[45] Nov. 30, 1976

[54] HYDRAULIC FLUIDS

[75] Inventors: **Gerald John Joseph Jayne; Herbert Frank Askew; Colin John Harrington**, all of Swindon, England

[73] Assignee: **Castrol Limited**, England

[22] Filed: **Sept. 24, 1974**

[21] Appl. No.: **508,842**

[30] Foreign Application Priority Data

Sept. 25, 1973 United Kingdom ..... 44905/73  
Dec. 14, 1973 United Kingdom ..... 58175/73

[52] U.S. Cl. .... **260/448.8 R; 252/78.3**

[51] Int. Cl.<sup>2</sup> .... **C07F 7/18**

[58] Field of Search ..... **260/448.8 R**

[56] References Cited

UNITED STATES PATENTS

3,336,227 8/1967 Göthel et al. .... **260/448.8 R X**

3,383,315 5/1968 Göthel et al. .... **260/448.8 R X**  
3,444,081 5/1969 Göthel et al. .... **260/448.8 R X**  
3,514,402 5/1970 Göthel et al. .... **260/448.8 R X**

Primary Examiner—Paul F. Shaver

Attorney, Agent, or Firm—Bacon & Thomas

[57]

## ABSTRACT

Novel glycol-substituted alkyl silanes useful as components of hydraulic fluids have the general formula:



wherein R, R<sup>1</sup>, R<sup>4</sup> and R<sup>5</sup> are specified substituents. Hydraulic fluids containing the glycol-substituted alkyl silanes are also described.

1 Claim, No Drawings

## HYDRAULIC FLUIDS

This invention relates to certain alkyl silane derivatives which are useful as components of hydraulic fluids and to hydraulic fluids containing such compounds particularly hydraulic fluids having high boiling point and vapour lock temperatures.

Hydraulic fluids based on glycol ethers have been used in, for example, vehicle brake and clutch systems for many years and still remain the most commonly used type of fluid. However, specifications of required quality standards laid down by hydraulic systems manufacturers and non-commercial organisations such as the Society of Automotive Engineers and the U.S. Department of Transportation have become progressively more severe. In particular, a need has arisen for fluids having higher boiling points and, more importantly, higher vapour lock temperatures both for the fluid as formulated by the manufacturers and also for the fluid in the presence of water. Glycol ether based fluids are known to be deficient in this respect due to the hygroscopicity of the fluid which results in the absorption of water from the atmosphere. This in turn reduces the boiling point and vapour lock temperature of the fluid and with extended use the water content of the fluid can build up to a level at which the boiling point and vapour lock temperatures are reduced to a dangerous extent. When subjected to heat, e.g. generated by heavy braking, the fluid may boil or vaporise to a sufficient extent to cause a serious brake malfunction.

Hydraulic fluids having low hygroscopicity have been developed, based on glycol esters, to deal with this problem. Such fluids are relatively insensitive to the effect of atmospheric moisture, but are more expensive than glycol ether based fluids and have certain technical disadvantages, e.g. their viscosity properties are inferior to those of glycol ether based fluids. Consequently, use of these low hygroscopicity fluids has been mainly limited to where the desirable properties such as high boiling point and vapour lock temperatures are deemed to outweigh their disadvantages. Other types of water insensitive fluids have also been developed. Nevertheless, manufacturers are still seeking new fluids which combine as many as possible of the desirable properties of both glycol ether based and low hygroscopicity fluids and, desirably, have even higher boiling points and/or vapour lock temperatures than the low hygroscopicity fluids.

Recently, there has emerged a growing tendency in vehicle design to use a single hydraulic system to operate equipment, such as power-steering, shock absorbers and brakes, which hitherto were provided with separate hydraulic systems. This has created serious problems in the formulation of suitable fluids. The mineral oil based fluids hitherto used in power-steering systems and shock absorbers are satisfactory with respect to the nitrile and chloroprene rubber used for the seals and gaskets in such systems but are highly detrimental to the natural and styrene/butadiene rubbers used in the construction of hydraulic brake and clutch systems. This results in excessive swelling of the latter seals which can lead to a serious malfunction of the brake or clutch system. Conversely, the fluids hitherto used in brake and clutch systems, which are normally based on glycols, glycol ethers and/or glycol ether esters, and which have operated satisfactorily in such systems, have a detrimental effect on the nitrile and

chloroprene rubber gaskets used in power-steering systems and shock absorbers which can also lead to malfunctioning. In the case of vehicle operation the characteristic of reliability in operation, which is generally desirable in all mechanical devices, is increased in importance to an absolutely essential requirement by virtue of safety considerations. The need has therefore arisen for a fluid which can be used satisfactorily in a central system controlling the operation of a number of different items of equipment.

We have now found certain alkyl silane derivatives which are useful as components of hydraulic fluids, for hydraulic brake and clutch systems and also for central hydraulic systems. These derivatives exhibit improved rubber swell properties with respect to a variety of natural and synthetic rubbers used in the construction of hydraulic systems and they are also relatively water insensitive.

Accordingly the present invention provides alkyl silane derivatives prepared by a process which comprises reacting a di- or tri-chlorosilane of the formula:



with a diol or polyol of the formula  $\text{HO}-\text{R}^4-\text{OH}$  and a glycol monoether of the formula:



wherein:

- R is an alkyl group;
- the or each group R<sup>2</sup> is a hydrogen atom or a methyl or ethyl group and each R<sup>2</sup> may be the same as or different from any other group R<sup>2</sup>;
- R<sup>3</sup> is an alkyl group;
- R<sup>4</sup> is the residue of a diol or polyol;
- n is an integer of from 1 to 10; and
- X is a chlorine atom or the group R.

In another aspect of the present invention there is provided a hydraulic fluid containing one or more alkyl silane derivatives prepared by the aforesaid process.

In the case of alkyl silane derivatives for use in hydraulic brake and clutch systems it is preferable for the groups R, R<sup>3</sup> to be relatively short chain alkyl groups, e.g. containing from 1 to 4, more preferably 1 or 2, carbon atoms, in order to minimise the rubber swelling effect on the seals and gaskets used in such systems. However when used in a central system it may be more desirable to effect a compromise between the requirements, often conflicting, for each of the various seal and gasket materials. In this case some, or all, of the groups R, R<sup>3</sup> may be longer chain alkyl groups, e.g. up to 6, or even 8, carbon atoms.

In yet another aspect of the present invention there is provided the process for the preparation of alkyl silane derivatives which comprises reacting a di- or tri-chlorosilane of the formula:



with a diol or polyol of the formula  $\text{HO}-\text{R}^4-\text{OH}$  and a glycol monoether of the formula:



wherein:

- a. R is an alkyl group;
  - b. the or each group R<sup>2</sup> is a hydrogen atom or a methyl or ethyl group and each R<sup>2</sup> may be the same as or different from any other group R<sup>2</sup>;
  - c. R<sup>3</sup> is an alkyl group;
  - d. R<sup>4</sup> is the residue of a diol or polyol;
  - e. n is an integer of from 1 to 10; and
  - f. X is a chlorine atom or the group R.

A dialkyl dichlorosilane may be reacted with a glycol of the formula:



and the glycol monoether. Alternatively an alkyl trichlorosilane may be reacted with a glycol of the formula:



and the glycol monoether.

Reaction of the glycol and glycol monoether with the alkyl chlorosilane may be carried out simultaneously in a single stage reaction. Such a single stage reaction may be more convenient but is more difficult to control and therefore sequential reaction is preferred, most preferably employing the glycol in the first stage.

In place of the glycol, a dihydroxy benzene, such as p-hydroxyphenol, or other diols such as neopentyl glycol, or a polyol such as trimethylol propane, pentaerythritol, dipentaerythritol, or a trihydroxy benzene may be used. In this case the product may bear one or more residual hydroxyl groups. Alternatively, sufficient chlorosilane may be used to react with all the hydroxyl groups of the polyol.

In the preparation of the hydraulic fluid components of the present invention, the reaction of a chlorosilane with a hydroxyl group may be carried out in the presence of an acid acceptor to neutralise liberated hydrogen chloride. Especially preferred acid acceptors are tertiary bases such as pyridine. To ensure substantially complete conversion it is usually preferred to use a slight, e.g. 10%, excess of the glycol monoether starting material. 55 60

The alkyl silane hydraulic fluid components may be used as an additive, as a base stock or as a component of a blend of base stocks. The proportions employed may therefore vary over a very wide range. When used as a base stock the alkyl silane derivatives will constitute the bulk of the hydraulic fluid, for example from 75 or 80 to 99% by weight, based on the total weight of the hydraulic fluid. The remainder of the hydraulic

fluid may be composed of conventional hydraulic fluid additives, as more fully described hereinafter, and/or small quantities of other hydraulic fluid base-stocks, as also more fully described hereinafter.

- 5 When used as a component of a blend of base stocks the total blend of base stocks will likewise constitute the bulk of the hydraulic fluid. In this case, the base stocks may be predominantly one or more alkyl silane derivatives blended with a lesser quantity of one or  
10 more other base stocks, of the type hereinafter described, so as to modify the properties of the alkyl silane derivatives. Thus the hydraulic fluid may contain, for example 55 to 70% by weight of one or more alkyl silane derivatives based on the total weight of the  
15 hydraulic fluid. Alternatively, one or more other base stocks may be modified by blending with a lesser quantity of alkyl silane derivatives so that the hydraulic fluid contains, e.g. from 20 to 40% by weight alkyl silane derivatives. In addition, a compromise between the  
20 properties of the alkyl silane derivatives and the other fluids may be effected by blending in approximately equal quantities to provide fluids containing from 40 to 55% alkyl silane derivatives.

When used to suppress the sensitivity of hydraulic fluids, and in particular the boiling point and vapour lock temperatures of the fluids, to water the glycol-substituted silanes are preferably used in amounts in the range of 20 to 55%, more preferably 20 to 40%. Alternatively but less preferably, an improvement can also be obtained using lower amounts of the glycol-substituted silanes, e.g. from 0.5 to 15 or 20% by weight based on the total weight of the hydraulic fluids. The bulk of such fluids will be constituted by one or more base stocks as hereinafter described.

- 35 When the alkyl silane derivatives are used as a component of a blend of base stocks the resulting hydraulic fluids may contain conventional hydraulic fluid additives in like manner as when the base stock substantially consists of the alkyl silane derivatives. Similarly,  
40 when used as an additive the alkyl silane derivatives may, if desired, be used in conjunction with conventional hydraulic fluid additives.

Base stocks with which the alkyl silane derivatives may be blended, or with which they may be used as additives, include glycols, glycol ethers, glycol esters, glycol orthoesters and borate esters. Glycol ether base stocks are well known and suitable examples thereof are those commonly used in hydraulic fluids. The preferred glycol ester base stocks are those having the general formula:



wherein R<sup>6</sup> is a straight or branched chain alkylene group containing at least 2, preferably 2 to 8, carbon atoms each R<sup>7</sup> is the same or different and is an alkyl radical containing from 1 to 4 carbon atoms or a phenyl radical, each R<sup>8</sup> is the same or different and is an ethylene, propylene or butylene group, each x is the same or different and is 0 or an integer of from 1 to 3, each R<sup>9</sup> is the same or different and is an ethyl or methyl group, each R<sup>10</sup> is the same or different and is an ethylene or propylene group and y is an integer, preferably an integer of from 1 to 3.

ger such that the total number of carbon atoms in the  $\text{+R}^{10}\text{O-}$  group is from 4 to 12, more preferably 4 to 9.

The dicarboxylic acid esters of formula I are described in British Patent Specification No. 1,083,324. Esters which may suitably be used in the present invention are the succinates, glutarates, adipates, azelates, sebacates, isosebacates and nylonates of methyl, ethyl, propyl and butyl monoethers of mono, di- and tri-ethylene glycols described in British Patent Specification No. 1,083,324, the nylonates, especially di mono-methyl ether of diethylene glycol nylonates, being particularly preferred.

The glycol di-esters of formula II are known compounds and the preferred glycol di-esters are the glycol dipropionates described in British Patent Specification No. 1,249,803. It is preferred that the hydraulic fluids comprise not more than 50% by weight of the glycol di-esters; the remainder, if any, of the carboxylic acid ester component being the esters of formula I.

Numerous varieties of borate ester base stocks are known and these may be depicted by the following general formula:



wherein each  $\text{R}^{11}$  is the same or different and is a straight or branched chain alkylene group, each  $\text{R}^{12}$  is the same or different and is an alkyl group, each  $p$  is the same or different and is an integer,  $q$  is an integer of from 2 to 6,  $\text{R}^{13}$  is the residue of a di- or poly-hydroxy organic compound having a number of reactive hydroxy groups equal to  $q$ , and each  $\text{R}^{14}$  is the same or different and is the residue of a di-hydroxy organic compound which residue is attached to each boron atom via an oxygen atom.

These borate esters are more fully described in British Patent Specification No. 1,341,901 to which reference may be made for further details.

Further base stocks which may be used are the glycol orthoesters described in British Patent Specification No. 1,330,468 having the general formula:



wherein  $\text{R}^{15}$  is a hydrogen atom, an alkyl radical containing from 1 to 5 carbon atoms, or the same as  $\text{OR}^{16}$ , each  $\text{R}^{16}$  is the same or different and each is an alkyl radical containing from 1 to 4 carbon atoms, an oxyalkylene glycol monoether radical, or a polyoxyalkylene glycol monoether radical containing from 2 to 20 alkylene oxy units, provided that at least one  $\text{R}^{16}$  is an oxyalkylene glycol monoether radical or a polyoxyalkylene glycol monoether radical; and  $\text{R}^{17}$  is an alkylene radical containing from 1 to 12 carbon atoms, provided that  $\text{R}^{15}$  is then the same as  $\text{OR}^{16}$  or  $\text{R}^{17}$  is the group  $\text{-O-R}^{18}\text{O-}$ , wherein each  $\text{R}^{18}$  is the same or different and each is an alkylene radical containing from 2 to 8 carbon atoms and  $z$  is an integer from 1 to 6. Reference may be made to British Patent Specification No. 1,330,468 for further details of such glycol orthoesters.

In a particularly preferred embodiment of the present invention the alkyl silane derivatives are used, as a base stock, in hydraulic fluids also comprising a small amount, e.g. 1 to 10% by weight, of a rubber swell modifier such as an ethylene glycol.

In another particularly preferred embodiment of the present invention the alkyl silane derivatives are used, either as an additive or as a component of a blend of base stocks, in hydraulic fluids comprising one or more glycol esters of foregoing formulae I and/or II or comprising a mixture of one or more glycol esters of foregoing formula I and/or II with one or more borate esters of foregoing formulae III to VII especially borate esters of formula III.

Typical additives which may be used in, or in conjunction with, the alkyl silane derivatives are lubricity additives selected from castor oil or castor oil treated in various ways, for example:

- 35 Firsts Castor Oil,  
Castor Oil to Specification DTD72  
Blown castor oil, i.e. castor oil blown with air or oxygen while being heated.
- 40 Special Pale Blown Castor Oil, i.e. a similarly blown castor oil, "Hydrin 4" i.e. a commercially available ethylene/oxide/propylene oxide treated castor oil.

Other lubricity additives which may be incorporated in hydraulic fluids in accordance with the present invention include borate esters e.g. tricresyl borate and phosphorus-containing esters, especially phosphates e.g. tricresyl phosphate.

The hydraulic fluids of the present invention may also include minor proportions of polyoxyalkylene glycols or ethers thereof e.g. those sold by Union Carbide Corporation under the Registered Trade Mark "Ucon", particularly those of the LB and HB series. Suitable examples of these polyoxyalkylene glycols and their ethers and esters are given in British Patent Specification No. 1,055,641. Other suitable lubricity agents are orthophosphate or sulphate salts of primary or secondary aliphatic amines having a total of from 4 to 24 carbon atoms, dialkyl citrates having an average of from 3½ to 13 carbon atoms in the alkyl groups, aliphatic dicarboxylic acids and esters thereof, specific examples being

- Diamylamine orthophosphate
- Dinonylamine orthophosphate
- Diamylamine sulphate
- 65 Dinonyl citrate
- Di(2-ethyl hexyl) citrate
- Polyoxyethylene sebacate derived from a polyoxyethylene glycol of M.W. 200

- Polyoxyethylene azelate derived from a polyoxyethylene glycol of M.W. 200  
 Polyoxyethylene adipate derived from a polyoxyethylene glycol of M.W. 200  
 Polyoxyethylene/polyoxypropylene glutarate derived from mixed polyoxyglycols of average M.W. of about 200  
 Glutaric acid  
 Azelaic acid  
 Sebatic acid  
 Succinic acid  
 Di ethyl sebacate  
 Di 2-ethyl hexyl sebacate  
 Di iso octyl azelate  
 Unsaturated aliphatic acids or their salts may also be used e.g. oleic acid or potassium ricinoleate.

Corrosion inhibitors which may be used in the present invention may be selected from heterocyclic nitrogen containing compounds, e.g. benzotriazole and benzotriazole derivatives such as those described in British Patent Specification No. 1,061,904 or mercapto benzothiazole. Many amines or derivatives thereof are also suitable as corrosion inhibitors, for example

- di n-butylamine  
 di n-amylamine  
 cyclohexylamine  
 morpholine  
 triethanolamine  
 and soluble salts thereof e.g. cyclohexylamine carbonate.

Phosphites are also good corrosion inhibitors e.g. Tri phenyl phosphite

Di isopropyl phosphite and certain inorganic salts may be incorporated e.g. sodium nitrate.

Other additives which may be included are antioxidants such as diarylamines e.g. diphenylamine, p,p'-dioctyl-diphenylamine, phenyl- $\alpha$ -naphthylamine or phenyl- $\beta$ -naphthylamine. Other suitable antioxidants are those commonly known as hindered phenols which are exemplified by

- 2,4-dimethyl-6-t-butyl phenol  
 2,6-di-t-butyl-4-methyl phenol  
 2,6-di-t-butyl phenol  
 1,1-bis (3,5-di-t-butyl-4-hydroxyphenyl)-methane  
 3,3',5,5'-tetra-t-butyl - 4 - 4' -dihydroxydiphenyl  
 3-methyl-4,6-di-t-butyl phenol  
 4-methyl-2-t-butyl phenol

Yet further additives which may be used are phenothiazine and its derivatives, for example those having alkyl, or aryl, groups attached to the nitrogen atom or to the aryl groups of the molecule.

Other additives which may be used include alkylene oxide/ammonia condensation products as corrosion inhibitors, for example the propylene oxide/ammonia condensation product described in British Patent Specification No. 1,249,803. Further lubricity additives which may be used are complex esters, such as that sold under the trade name Reoplex 641 and also described in British Patent Specification No. 1,249,803. Moreover, long chain (e.g. C<sub>10-18</sub>) primary amine corrosion inhibitors and polymerised quinoline resin antioxidants, as described in Specification No. 1,249,803, may be used, examples of such amines and resins being the commercially available materials Armeen 12D and Agerite resin D respectively.

Conventional additives such as those hereinbefore described are normally employed in small amounts such as 0.05 to 10%, for example, 0.1 to 2% by weight.

We have found that tertiary amines have advantages over primary and secondary amines as corrosion inhibitors such that hydraulic fluids in accordance with the present invention containing tertiary amines show less tendency to gel, especially in the case of hydraulic fluids wherein R<sup>19</sup> is as the group R<sup>1</sup>. Thus, a particularly preferred aspect of the present invention provides hydraulic fluids containing one or more tertiary amines, or derivatives thereof, having the general formula:



wherein each R<sup>19</sup> is the same or different and is an alkyl group, preferably containing from 1 to 6 carbon atoms, an aryl, alkaryl or aralkyl group, preferably containing from 6 to 12 carbon atoms or a group having the general formula:



wherein the, or each, group R<sup>20</sup> is a straight or branched chain alkylene group, preferably an ethylene, propylene or butylene group, R<sup>21</sup> is a hydrogen atom or an alkyl group preferably containing from 1 to 6 carbon atoms and m is an integer of from 1 to 6, or any two groups R<sup>19</sup> may be taken together to form a cyclic system provided that if the nitrogen atom is thereby rendered tertiary the third group R<sup>19</sup> is absent.

When two of the groups R<sup>19</sup> in the above general formula are taken together, the cyclic system so formed preferably contains 4 to 6 carbon atoms in the ring. Further hetero atoms such as oxygen and nitrogen may also be contained in the ring as, for example, in tertiary amines derived from morpholine and piperazine respectively; it is desirable however that any further nitrogen hetero atoms should also be tertiary as in 1,4-dimethyl piperazine. Examples of tertiary amines in accordance with the above general formula wherein the two groups R<sup>19</sup> taken together render the nitrogen atom tertiary, the third group R<sup>19</sup> thus being absent, are pyridine and quinoline.

Especially preferred tertiary amines for use in the hydraulic fluids of the present invention are triethylamine, triethanolamine, triphenylamine and amines having the formula:



amines of said formula being commercially available under the trade name PROPYLAN A 350.

The tertiary amines may be employed in an amount of from 0.05 to 3.00 percent by weight based on the total weight of the hydraulic fluid.

Regardless of precise composition it is highly desirable that the hydraulic fluids of the present invention have a kinematic viscosity at -40° C. of not more than 5,000 cSt, especially not more than 2,000 cSt. It is also

desirable that the hydraulic fluids have a boiling point of at least 260° C.

In a particular aspect of the present invention there is provided a hydraulic system which contains, as the functional fluid, a hydraulic fluid as hereinbefore described.

In a further particular aspect of the present invention there is provided a method of operating a hydraulic system which comprises introducing into the hydraulic system a hydraulic fluid as hereinbefore described and transmitting power by applying pressure to the hydraulic fluid.

The present invention will now be illustrated with reference to the following Examples:

#### EXAMPLE 1

Triethylene glycol (150g., 1.0m) and pyridine (158g., 2.0m), were mixed and the resulting mixture added to dimethyl dichloro silane (258g., 2.0m) dissolved in toluene (3.01) over a period of 12 minutes. During the addition a dense white precipitate was formed and an exotherm was noted. The temperature

of the reaction mixture was kept below 42° C. during the addition.

The reaction mixture was then heated to about 100° C for 4 hours and then allowed to cool. To the resulting first stage product was added a mixture of triethylene glycol monomethyl ether (361g., 2.2m) and pyridine (174g., 2.2m) over a period of 20 minutes during which an exotherm was noted. During the exotherm the temperature was kept below 35° C., but thereafter the reaction mixture was heated to about 100° C., for 4 hours. The resulting product was allowed to cool and was then filtered, the filter cake being washed with further toluene. The solvent (toluene) was removed from the filtrate using a rotary evaporator and the product stripped to 180° C./0.05 torr. The final product (yield 333.0g.) was a clear, very pale yellow liquid containing 11.1% by weight Si and 0.03% by weight Cl (theory 9.5% and 0 respectively).

#### EXAMPLES 2 to 25

Further preparations were carried out in a similar manner as in Example 1, salient differences being summarised in the following Table 1.

TABLE 1

| EXAMPLE NO | DIOL OR POLYOL                   | PREPARATION OF BIS-SILANES<br>REACTION MIXTURE COMPONENTS |                         |                      | PYRIDINE (g) |
|------------|----------------------------------|-----------------------------------------------------------|-------------------------|----------------------|--------------|
|            |                                  | GLYCOL MONOETHER                                          | ALKYL CHLORO SILANE     | SOLVENT <sup>a</sup> |              |
| 2          | diethylene glycol 106g           | triethylene glycol mono-methyl ether 361g                 | dimethyl dichloro 258g  | 2.5L                 | 158 + 174    |
| 3          | PHG 200 <sup>a</sup> 198g        | "                                                         | "                       | 2.5L <sup>b</sup>    | "            |
| 4          | triethylene glycol 750g          | triethylene glycol mono-methyl ether 1805g                | dimethyl dichloro 1290g | 15L                  | 790 + 870    |
| 5          | 1,2-propylene glycol 76g         | triethylene glycol mono-methyl ether 361g                 | dimethyl dichloro 258g  | 2.5L                 | 158 + 174    |
| 6          | PPG 425 <sup>b</sup> 425g        | "                                                         | "                       | "                    | "            |
| 7          | PEG 200 <sup>a</sup> 297g        | diethylene glycol mono-methyl ether 496g                  | di-methyl dichloro 387g | 3.0L                 | 237 + 261    |
| 8          | PEG 200A 198g                    | ethylene glycol mono-methyl ether 167g                    | dimethyl dichloro 258g  | 2.5L                 | 158 + 174    |
| 9          | PEG 200 <sup>a</sup> 200g        | dipropylene glycol mono-methyl ether 326g                 | dimethyl dichloro 258g  | 2.5L                 | 158 + 174    |
| 10         | PPG 425 <sup>b</sup> 425g        | "                                                         | "                       | "                    | "            |
| 11         | PPG 150 <sup>c</sup> 300g        | dipropylene glycol mono-methyl ether 651g                 | dimethyl dichloro 516g  | 2.5L                 | 316 + 348    |
| 12         | 1,1,1-trimethylol propane 134.2g | triethylene glycol mono-methyl ether 541g                 | dimethyl dichloro 387g  | 1.0L + 2.0L          | 237 + 261    |

| EXAMPLE NO | REACTION CONDITIONS |                 | STRIPPING CONDITIONS |      | ANALYSIS  |                                |                                |
|------------|---------------------|-----------------|----------------------|------|-----------|--------------------------------|--------------------------------|
|            | FIRST STAGE hrs.    | SECOND STAGE °C | °C                   | torr | YIELD (g) | % Si <sup>L</sup> <sup>M</sup> | % Cl <sup>L</sup> <sup>M</sup> |
| 2          | 4/100               | 4/100           | 190                  | 0.05 | 311       | 9.49 (10.2)                    | 0 (0)                          |
| 3          | "                   | "               | 190                  | 0.05 | 343.8     | 7.74 (8.78)                    | 0.14 (0)                       |
| 4          | "                   | " <sup>k</sup>  | 176                  | 0.3  | 2508.1    | 8.81 (9.5)                     | 0.04 (0)                       |
| 5          | 4/100               | 4/100           | 171                  | 0.1  | 389.9     | 8.72 (10.8)                    | 0.04 (0)                       |
| 6          | "                   | "               | 182                  | 0.1  | 777.5     | 5.15 (6.48)                    | 0.04 (0)                       |

TABLE 1-continued

|    |       |       |     |      |       |        |      |
|----|-------|-------|-----|------|-------|--------|------|
| 7  | 4/100 | 4/100 | 180 | 0.05 | 479.7 | 10.69  | 0.03 |
| 8  | "     | "     | 160 | 0.05 | 322.8 | 12.07  | 0.09 |
| 9  | "     | "     | 167 | 0.15 | 442.5 | 8.6    | 0.12 |
| 10 | "     | "     | 183 | 0.4  | 580.7 | 5.9    | 0.11 |
| 11 | "     | "     | 146 | 0.1  | 795.9 | (6.73) | (0)  |
| 12 | 6/100 | 4/100 | 171 | 0.1  | 606.0 | 5.8    | >0.1 |
|    |       |       |     |      |       | (10.0) | (0)  |
|    |       |       |     |      |       | 8.9    | 0.11 |
|    |       |       |     |      |       | (10.6) | (0)  |

| EXAMPLE<br>NO | REACTION MIXTURE COMPONENTS               |                                                      |                                        |                      |                              | PYRIDINE<br>(g) |
|---------------|-------------------------------------------|------------------------------------------------------|----------------------------------------|----------------------|------------------------------|-----------------|
|               | DIOL OR<br>POLYOL                         | GLYCOL                                               | ALKYL<br>CHLORO<br>SILANE              | SOLVENT <sup>b</sup> |                              |                 |
| 13            | Neopentyl<br>glycol<br>208g               | diethylene<br>glycol mono-<br>methyl ether<br>528g   | dimethyl<br>dichloro<br>516g           | 2.5L                 | 316<br>+<br>348              |                 |
| 14            | PEG 200 <sup>a</sup><br>200g              | diethylene<br>glycol mono-<br>ethyl ether<br>294g    | dimethyl<br>dichloro<br>258g           | 2.5L                 | 158<br>+<br>174              |                 |
| 15            | Quinol<br>110g                            | triethylene<br>glycol mono<br>methyl ether<br>361g   | "                                      | 2.0L <sup>c</sup>    | 158<br>+<br>173              |                 |
| 16            | ethylene<br>glycol<br>62g                 | diethylene<br>glycol mono-<br>methyl ether<br>528g   | monomethyl<br>trichloro<br>299g        | 2.5L                 | 158<br>+<br>348              |                 |
| 17            | neopentyl<br>glycol<br>104g               | "                                                    | "                                      | 3.0L                 | "                            |                 |
| 18            | "                                         | "                                                    | "                                      | 2.5L                 | "                            |                 |
| 19            | 1,2-propy-<br>lene<br>glycol<br>76g       | "                                                    | "                                      | 2.5L <sup>c</sup>    | "                            |                 |
| 20            | PPG 150<br>300g.                          | triethylene<br>glycol mono-<br>methyl ether<br>722g. | dimethyl<br>dichloro<br>516 g.         | 2.5L                 | 316<br>+<br>348              |                 |
| 21            | EG<br>124g.                               | "                                                    | "                                      | 2.5L <sup>c</sup>    | "                            |                 |
| 22            | 1,2-propy-<br>lene<br>glycol<br>300g.     | "                                                    | "                                      | 2.5L <sup>c</sup>    | 484 <sup>a</sup><br>+<br>532 |                 |
| 23            | PEG<br>200g.                              | diethylene<br>glycol mono-<br>ethyl ether<br>132g    | dimethyl<br>dichloro<br>258g           | 2.5L                 | 158<br>+<br>174              |                 |
|               |                                           | dipropylene<br>glycol mono-<br>methyl ether<br>148g. |                                        |                      |                              |                 |
| 24            | triethyl-<br>glycol<br>300g               | triethylene<br>glycol mono-<br>methyl ether<br>820g  | dimethyl<br>dichloro<br>516g           | 1.5L                 | None <sup>a</sup>            |                 |
| 25            | 1,1,1,<br>trimeth-<br>ylopropane<br>134g. | diethylene<br>glycol mono-<br>methyl ether<br>792g   | mono-<br>methyl<br>trichloro<br>448.5g | 1.0L<br>+<br>2.0L    | 237<br>+<br>521              |                 |

| EXAMPLE<br>NO | REACTION<br>CONDITIONS |                 | STRIPPING<br>CONDITIONS |      | YIELD<br>(g) | ANALYSIS          |                   |
|---------------|------------------------|-----------------|-------------------------|------|--------------|-------------------|-------------------|
|               | FIRST<br>STAGE         | SECOND<br>STAGE | ° C                     | torr |              | % Si <sup>b</sup> | % Cl <sup>b</sup> |
| 13            | 4/100                  | 4/100           | 152                     | 0.05 | 491.8        | 8.22<br>(12.3)    | <0.1<br>(0)       |
| 14            | "                      | "               | 165                     | 0.05 | 462.4        | 5.3<br>(9.65)     | <0.1<br>(0)       |
| 15            | 4/100                  | 4/100           | 180                     | 0.1  | 481.4        | 13.1<br>(10.2)    | 0.16<br>(0)       |
| 16            | 4/100                  | 4/100           | 188                     | 0.1  | 340.7        | 9.08<br>(9.0)     | 0.1<br>(0)        |
| 17            | "                      | "               | 190                     | 0.1  | 238.3        | 7.5<br>(8.45)     | <0.05<br>(0)      |
| 18            | "                      | "               | 174                     | 0.1  | 440.9        | 8.41<br>(8.44)    | 0.05<br>(0)       |
| 19            | "                      | "               | 152                     | 0.02 | 456.9        | 9.61<br>(8.8)     | 0.07<br>(0)       |
| 20            | "                      | "               | 160                     | 0.1  | 653.3        | 10.1<br>(9.5)     | <0.1<br>(0)       |
| 21            | "                      | "               | 177                     | 0.1  | 675.4        | 10.7<br>(11.1)    | <0.1<br>(0)       |

TABLE 1-continued

|    |       |        |     |                 |            |          |
|----|-------|--------|-----|-----------------|------------|----------|
| 22 | 4/80  | 4/80   | 170 | 0.5 to 1.0798.7 | 6.8        | 0.13     |
| 23 | 4/100 | 4/100  | 169 | 0.05 348.8      | (9.5) 9.77 | (0) <0.1 |
| 24 | "     | 12/100 | 170 | 0.1 895.0       | (9.65) 7.5 | (0) <0.1 |
| 25 | 6/100 | 4/100  | 190 | 0.1 650.4       | (9.5) 5.6  | (0) <0.1 |
|    |       |        |     |                 | (8.25)     | (0)      |

## FOOTNOTES TO TABLE 1

\*PEG 200 is a commercially available mixture of polyethylene glycols having an average molecular weight of about 200.

\*PPG 425 is a commercially available mixture of polypropylene glycols having an average molecular weight of about 425.

\*PPG 150 is a commercially available mixture of polypropylene glycols having an average molecular weight of about 150.

\*Toluene, except in examples 12 and 25 when diethylene glycol diether (1.0L) used initially and a further 2.0L of toluene added prior to second stage.

\*Further 0.5L added during second stage to aid stirring.

\*Further 0.15L added during second stage to aid stirring.

\*Quinol/pyridine mixture dissolved in further 0.4L toluene prior to addition to silane.

\*Further 0.25L toluene added during second stage to aid stirring.

\*Glycol/pyridine mixture added to silane over 1-3/4 hr.

\*Glycol monoether/pyridine mixture added to 1st stage over 2 hrs.

\*Due to difficulties in the elemental analysis of organic silicon compounds values obtained for Si content are commonly low.

\*Calculated figures in parenthesis.

\*N,N-dimethylaniline used in place of pyridine.

\*Carbon tetrachloride used in place of toluene.

\*HCl blown out with N<sub>2</sub>.

IR Spectra of the products of the foregoing examples were all found to be consistent with the expected product being obtained.

To determine the suitability of the products of the foregoing examples for use in hydraulic fluids the following tests were carried out.

a. Kinematic viscosities at -40°, in centistokes, were measured in the manner set forth in the SAE J1703c

After the test, the percentage volume increase of each of the rubber specimens was measured.

The results of these tests are set out in the following Table 2. In addition, the hydrolytic stability of a number of products were tested in accordance with the Water Tolerance tests as set out in the SAE J1703c specification, all products so tested satisfying the stability standards required by this test.

TABLE 2

| Product Tested<br>Example No. | Viscosity<br>(-40° C) | Rubber Swell      |                                 |                   | Wet Vapour Lock<br>Temperatures (° C) |
|-------------------------------|-----------------------|-------------------|---------------------------------|-------------------|---------------------------------------|
|                               |                       | Natural<br>rubber | Styrene/<br>Butadiene<br>rubber | Nitrile<br>Rubber |                                       |
| 1                             | 829                   | ~ 5               | ~ 21                            | ~ 16              | 215                                   |
| 2                             | 321                   | 8.2               | 32.8                            | 33.8              | 249                                   |
| 3                             | 1993                  | 3.1               | 12.7                            | 13.0              |                                       |
| 4                             | 765                   | 4.8               | 17.0                            | 18.8              |                                       |
| 5                             | (low)                 | 12.4              | 37.3                            | 39.0              | 235                                   |
| 6                             | 4172                  | 8.8               | 18.5                            | 7.3               | 176                                   |
| 7                             | 1832                  | 4.3               | 12.1                            | 6.8               | 226                                   |
| 8                             | 1549                  | 4.9               | 12.5                            | 6.0               | 174                                   |
| 9                             | 1712                  | 16.1              | 22.5                            | 5.5               | 212                                   |
| 10                            | 16439                 | 17.6              | 21.0                            | -5.0              | 237                                   |
| 11                            | 362.3                 | 49.7              | 47.1                            | 3.6               |                                       |
| 12                            | 515.3                 | 23.8              | 39.6                            | 33.0              | 225                                   |
| 13                            | 77.5                  | 35.5              | 59.7                            | 38.9              | 187                                   |
| 14                            | 1015                  | 10.8              | 21.7                            | 11.7              |                                       |
| 15                            | 2261                  | 5.3               | 23.9                            | 32.5              |                                       |
| 16                            | 383                   | 4.3               | 15.0                            | 23.7              |                                       |
| 18                            | 249                   | 9.5               | 25.1                            | 42.8              |                                       |
| 19                            | 589                   | 12.8              | 6.2                             | 21.7              |                                       |
| 20                            | 379                   | 11.6              | 24.9                            | 26.4              | 230                                   |
| 21                            | 247                   | 11.6              | 32.1                            | 39.3              | 247                                   |
| 22                            |                       | 10.9              | 19.0                            | 20.8              | 230                                   |
| 23                            |                       | 7.5               | 16.9                            | 6.4               | 201                                   |
| 24                            | 780                   | 4.7               | 13.4                            | 22.6              |                                       |
| 25                            | 986                   | 6.5               | 13.6                            | 21.5              | 208                                   |

specification.

b. Samples were subjected to the D.O.T. Humidity test according to the procedure set forth in the FMVSS 116 specification and the vapour lock temperatures of the samples were measured. The vapour lock temperatures were determined in the manner described in British Patent Specification No. 1,341,910.

c. Rubber Swell properties were measured by placing 1 inch square by 3 mm. thick rubber specimens in 60 ml jars each containing 50 ml test fluid for a period of 3 days during which the temperature was maintained at 70° C. for the nitrile and natural rubber specimens and at 120° C. for the styrene/butadiene rubber specimens.

55 We claim:

1. Alkyl silane derivatives prepared by the process comprising reacting a di- or tri-chlorosilane of the formula:



with a diol or polyol of the formula HO—R<sup>4</sup>—OH and a glycol monoether of the formula:



wherein

- a. R is an alkyl group;
- b. the or each group R<sup>2</sup> is a hydrogen atom or a methyl or ethyl group and each R<sup>2</sup> may be the same as or different from any other group R<sup>2</sup>;
- c. R<sup>3</sup> is an alkyl group;
- d. R<sup>4</sup> is the residue of a diol or polyol;
- e. n is an integer of from 1 to 10; and
- f. X is a chlorine atom or the group R.

2. Alkyl silane derivatives as claimed in claim 1 wherein the reaction of the di- or tri-chlorosilane with the diol or polyol and glycol monoether is carried out simultaneously in a single stage reaction.

3. Alkyl saline derivatives as claimed in claim 1 wherein the reaction of the di- or tri-chlorosilane with the diol or polyol and glycol monoether is carried out as a two stage reaction.

4. Alkyl silane derivatives as claimed in claim 3 wherein the first stage reaction is the reaction of the di- or tri-chlorosilane with the diol or polyol.

5. Alkyl silane derivatives as claimed in claim 1 wherein the reaction is carried out in the presence of an acid acceptor to neutralize liberated hydrogen chloride.

6. Alkyl saline derivatives as claimed in claim 1 wherein the di- or tri-chlorosilane is reacted with a glycol or a dihydroxy benzene.

7. Alkyl silane derivatives as claimed in claim 6 wherein the di- or tri-chlorosilane is reacted with neopentyl glycol.

8. Alkyl silane derivatives as claimed in claim 1 wherein the di- or tri-chlorosilane is reacted with trimethylol propane, pentaerythritol, dipentaerythritol or a tri-hydroxy benzene.

9. Alkyl silane derivatives as claimed in claim 1 wherein a dialkyl dichlorosilane is reacted with a glycol of the formula HO—CH<sub>2</sub>—CH<sub>2</sub>—O—<sub>n</sub>H and the glycol monoether.

10. Alkyl silane derivatives as claimed in claim 1 wherein an alkyl trichlorosilane is reacted with a glycol of the formula HO—CH<sub>2</sub>—CH<sub>2</sub>—O—<sub>n</sub>H and the glycol monoether.

\* \* \* \* \*